

# UNITED STATES PATENT OFFICE.

LEON CAMMEN, OF TUCKAHOE, NEW YORK.

## CENTRIFUGAL CASTING.

No Drawing.

Application filed February 24, 1922. Serial No. 539,031.

To all whom it may concern:

Be it known that I, LEON CAMMEN, a citizen of the United States, and resident of the village of Tuckahoe, Westchester County, 5 State of New York, have invented certain useful Improvements in Centrifugal Castings, of which the following is a specification.

The present is a companion application 10 to the application by the same inventor entitled Casting tubular goods, filed July 18, 1921, Ser. No. 485,698, Div. 3, Room 175, in which all claims have been found allowable. Like the former application, it refers 15 to the casting by centrifugal means of goods from metals which chill very rapidly, such as Monel metal and various steels.

All attempts to cast them into shapes of 20 comparatively thin sections have failed because the metal chilled too rapidly, often before it had time to form into a pipe. The present invention provides a process wherein the mold is heated to a high temperature, close to the melting point of the metal to be 25 poured. This hot mold is then placed into a metal frame or sheath, to give it the necessary mechanical support and is, with its frame or sheath, subjected to centrifugal spinning, whereupon the metal is poured

into the mold. The molten metal coming 30 in contact with the very hot mold does not lose its heat with the same speed as when it hits a cold mold, and enough time becomes available to form a good tube.

The temperature to which the mold has 35 to be heated should be close to the melting point of the metal which means in practice from 300 to 800 deg. Fahr. below it, depending on conditions in each case. The proper selection of the temperature in each case 40 is a matter which a good foundryman with an understanding of the present process can easily handle.

I claim:

A process of centrifugal casting comprising 45 the following steps: heating the mold to a temperature close to the melting point of the metal to be poured, inserting the mold into a metal sheath to give it mechanical strength, subjecting the whole to centrifugal 50 spinning, and pouring molten metal into the mold.

Signed in New York, in the county and State of New York, February 23, 1922.

LEON CAMMEN.

Witness:

ERNEST HARTFORD.